

106/84

1,393,346

## UNITED STATES PATENT OFFICE.

FRANK J. COOK, OF CLEVELAND, OHIO.

## INSULATING COMPOSITION OF MATTER.

1,393,346.

Specification of Letters Patent. Patented Oct. 11, 1921.

No Drawing.

Application filed August 19, 1920. Serial No. 404,650.

*To all whom it may concern:*

Be it known that I, FRANK J. COOK, a citizen of the United States, residing at Cleveland, in the county of Cuyahoga and State of Ohio, have invented a certain new and useful Improvement in Insulating Composition of Matter, of which the following is a full, clear, and exact description.

The present invention relates to a composition of material which is a non-conductor of electricity, and is a poor conductor of heat so far as radiation of heat to the air or atmosphere is concerned, but does act as a conductor of heat between metals.

The composition of material has certain valuable properties, as will appear more fully as the description proceeds, which makes it eminently fitted for use as an insulating composition, in which electric resistance wire is embedded.

The composition of matter comprises as its ingredients pulverized soap-stone, or talc, pulverized feldspar, pulverized flint, and ball clay, all of which materials, as before stated, being in finely divided condition, are thoroughly mixed with each other and to the mixture there is added a suitable quantity of a solution of sodium silicate, which is preferably a 50% solution.

The proportions of the ingredients may be varied to meet varied requirements, but as a very satisfactory composition, I may state the following proportions:

|    |                                                       |          |
|----|-------------------------------------------------------|----------|
| 35 | Soapstone -----                                       | 10 parts |
|    | Feldspar -----                                        | 1 part   |
|    | Flint -----                                           | 1 part   |
|    | Ball clay -----                                       | 1 part   |
|    | Solution sodium silicate to make desired consistency. |          |

The predominating ingredient is soap-stone, and this ingredient supplies to the composition the quality of absorbing heat and passing it on to a metal with which it is in contact. The other ingredients enhance the baking and expanding properties of the composition as later explained.

The sodium silicate acts as a binder for the materials and while I prefer to use silicate of soda, other soluble silicates such as sodium silicate of potash may be used.

The quantity of silicate of soda solution added is sufficient to make a plastic mass or thick paste, in which condition the composition is ready for use.

When the composition has been placed

and formed for its ultimate use, the composition is permitted to dry at a suitable temperature and in practice I find a temperature of 200° F. is about right. After thorough drying the temperature is raised to approximately 250° F. at which temperature the baking is continued until the composition is thoroughly baked and hardened, which requires approximately two hours although the baking time varies with the quantity and thickness of the material.

The composition of matter which has been described is particularly useful for use in connection with the laying of electric resistance wires upon a suitable support, and embedding such wires to prevent rapid radiation of the heat to the atmosphere, and at the same time serving to hold the resistance wire in its laid position, thus maintaining the wires in their proper spaced relationship, and preventing them from moving from their fixed position.

When the resistance wire is applied so as to heat a metal body, as for instance an iron pipe or other metal structure, a thin coating of the material mixed as before stated is applied to the metal surface, thus filling in any irregularities in the surface, and this coating is dried out and baked as before stated. The resistance wire is then laid in place upon the coating, and a second coating is applied over the wires, forming a layer of suitable thickness and the article is again subjected to the drying and baking process.

If necessary, a third coating may be added, dried out and baked, as before stated. It will be understood that it is necessary and desirable that the electric resistance wire be completely embedded in the plastic material in order to prevent radiation to the air.

The composition of matter which has before been described has the peculiar property of conducting the heat from the electrical resistance wire, and passing it on to the metal with which it is in contact, but the radiation of heat through the described composition of matter from the electrical resistance wire to the atmosphere is very slow, particularly as compared with the radiation of heat to the metal object with which it is in contact. This property of the composition is very important, inasmuch as due to its plastic qualities when applied, it permits all the interstices in the surface of the metal to be filled, and when the wire is embedded

60

65

70

75

80

85

90

95

100

105

110

in the plastic material, and subsequently baked, the heat from the wire when a current is passed through the same is evenly applied and distributed over all the metal surface 5 with which the plastic material is in contact.

The composition of matter when properly applied and baked has a degree of expansion, so that the composition expands with the heating of the metal to which it is applied 10 and contracts with it when cooling, thus being free from cracking or blistering.

The material is highly resistant to the electric current, so that leakage of current between adjacent coils or parallel strips of the 15 resistance wire or material is prevented.

Where an electrical conductor, be it of resistance wire or a good conductor, is placed upon a porcelain support or support of refractory material, the composition which has 20 been described may be employed to embed the wire in the grooves of the porcelain insulator, in which event it is not necessary to apply a preliminary coating of the material, but simply apply a coating to the insulator 25 after the wire is laid, baking the same, and

if necessary or desired, applying a second coat so as to completely embed the wires.

While the composition has been described with particular reference to its use in connection with electrical resistance wire, it will 30 be understood that the use of it is not limited in this particular, but it is adaptable for use wherever its heat insulating and electrical insulating properties may be desired or advantageous.

Having described my invention, I claim:—

1. A composition of matter comprising substantially ten parts of pulverized soapstone, one part of feldspar, one part of flint, one-half part of ball clay, to which is added 40 a binder.

2. A composition of matter comprising substantially ten parts of pulverized soapstone, one part of feldspar, one part of flint, one-half part of ball clay, and a binder con- 45 sisting of sodium silicate.

In testimony whereof, I hereunto affix my signature.

FRANK J. COOK.